

## UNITED STATES PATENT OFFICE

2,513,935

## ALLOY STEELS

Geoffrey Thomas Harris, Sheffield, England, assignor, by mesne assignments, to William Jessop & Sons Limited, Sheffield, England, a British company

No Drawing. Application December 10, 1948, Serial No. 64,703. In Great Britain December 13, 1947

4 Claims. (Cl. 75—126)

1

This invention relates to alloy steels and has for its object the provision of an alloy steel having good creep strength and resistance to scaling at temperatures in the region of 600° C.

The invention is particularly concerned with improving the creep strength and resistance to scaling of alloy steels of the kind frequently referred to as stainless "irons." The creep strength of such stainless irons, which do not normally contain molybdenum or tungsten can, as is known, be improved to a limited extent by the addition of molybdenum or tungsten. For example the following table shows three alloys and the stress required to produce a minimum creep rate of  $10^{-6}$  per hour at a temperature of 550° C.

## Stress required

|                                   |     |
|-----------------------------------|-----|
| 12% chromium-iron                 | 2.4 |
| 12% chromium-iron+0.5% molybdenum | 3.7 |
| 12% chromium-iron+3% tungsten     | 6.3 |

However steels made in accordance with the present invention, as hereinafter described, require a stress of 15 tons per square inch to produce a minimum creep rate of  $10^{-6}$  per hour at a temperature of 550° C.

According to my invention an alloy comprises the following ingredients within the ranges mentioned:

|                         | Per cent |
|-------------------------|----------|
| Carbon                  | 0.05-0.5 |
| Manganese               | 0.05-1.0 |
| Silicon                 | 0.05-1.0 |
| Chromium                | 9.0-15.0 |
| Molybdenum              | 0.2-1.2  |
| Vanadium                | 0.2-2.0  |
| Niobium and/or tantalum | 0.05-1.5 |

the remainder being iron and usual impurities.

Tungsten up to 1% may also be added.

Since in niobium ores tantalum is usually present and as it is difficult to separate niobium and tantalum, in practice small amounts of tantalum are usually present in association with niobium. For example, commercial ferro-niobium contains roughly 65% niobium and up to 5% tantalum. Thus my invention, so far as the addition of niobium is concerned includes the presence of small amounts of tantalum usually found with niobium. It also includes the re-

placement of niobium in whole or in part by tantalum.

The following is an example of a particular alloy in accordance with the invention:

|             | Per cent |
|-------------|----------|
| Carbon      | 0.16     |
| Manganese   | 0.27     |
| Silicon     | 0.32     |
| 10 Chromium | 11.1     |
| Molybdenum  | 0.63     |
| Vanadium    | 0.74     |
| Niobium     | 0.17     |

15 the remainder being iron and usual impurities.

Tests on this alloy gave the following results. Bar material was forged and heat treated by quenching in oil from 1200° C. followed by tempering at 720° C.

20 A creep test under a stress of 10 tons per square inch at a temperature of 650° C. gave a minimum creep rate, that is the constant rate of creep attained in the stage of secondary creep, of approximately  $1.9 \times 10^{-5}$  per hour. This creep rate produced under a stress of 10 tons per square inch is produced in previously known non-austenitic steels by stresses in the range of 2 to 8 tons per square inch. A further creep test on the alloy under a stress of 15

25 tons per square inch at a temperature of 550° C. gave a minimum creep rate of approximately  $10^{-6}$  per hour. The alloy also possesses superior scaling resistance properties to those shown by the stronger type of non-austenitic alloy, and the alloy therefore combines high scaling resistance

30 with high creep strength. The heat treatment can be varied to suit requirements and even higher creep strengths can be attained by quenching from a temperature higher than 1200° C., whilst a somewhat lower creep strength combined with greater ductility and toughness can be obtained by quenching from lower temperature.

35 Alloy steels according to this invention are particularly useful for the manufacture of articles in which a good creep strength and resistance to scaling at high temperatures is required. Such articles are, for example, rotors and blades for gas turbines.

40 45 Having thus described my invention, what I

claim as new and desire to secure by Letters Patent is:

1. Alloy steels comprising the following ingredients in the proportions specified

|            | Per cent   |
|------------|------------|
| Carbon     | About 0.16 |
| Manganese  | About 0.27 |
| Silicon    | About 0.32 |
| Chromium   | About 11.1 |
| Molybdenum | About 0.63 |
| Vanadium   | About 0.74 |
| Niobium    | About 0.17 |

the remainder being iron and usual impurities.

2. An alloy steel comprising the following ingredients within the ranges specified: carbon .05 to .5%, manganese and silicon each within the range of .05% to 1.0%, chromium 9 to 15%, molybdenum 0.2% to 1.2%, vanadium 0.2 to 2%, and at least one element selected from the group consisting of niobium and tantalum .05 to not over 1.5%, substantially all of the remainder being iron and usual impurities, said composi-

tion having a high creep strength and resistance to scaling at temperatures of the order of 600° C.

3. An alloy steel as defined in claim 2 containing tungsten up to one per cent.

4. An alloy steel of good creep strength and resistance to scaling at high temperatures comprising the following ingredients in approximately the following proportions: carbon .16%, manganese and silicon each .3%, chromium 11%, molybdenum .63%, vanadium .75% and at least one element selected from the group consisting of niobium and tantalum .17%, substantially all the remainder being iron and usual impurities.

GEOFFREY THOMAS HARRIS.

#### REFERENCES CITED

The following references are of record in the file of this patent:

#### UNITED STATES PATENTS

Number Name Date  
1,687,486 Armstrong Oct. 16, 1928